# EUROPEAN PATENT SPECIFICATION

(11) **EP 1 707 617 B1**
(45) Date of publication and mention of the grant of the patent: **15.03.2017**
(21) Application number: 05709443.5
(22) Date of filing: 28.01.2005
(51) Int. Cl.: C10M 169/04, C10M 105/38, C10M 105/40, C10M 129/10, C10M 133/38, C10M 133/44, C10M 135/10, C10M 159/24, C10N 10/04, C10N 20/00, C10N 20/02, C10N 30/00, C10N 30/02, C10N 30/06, C10N 30/08, C10N 30/10, C10N 30/12, C10N 40/04, C10N 40/08, C10N 40/20

(54) **BIODEGRADABLE LUBRICATING OIL COMPOSITION**
BIOLOGISCH ABBAUBARE SCHMIERÖLZUSAMMENSETZUNG
COMPOSITION D'HUILE DE LUBRIFICATION BIODÉBRADABLE

(30) Priority: 30.01.2004 JP 2004024291
(43) Date of publication of application: 04.10.2006
(73) Proprietor: IDEMITSU KOSAN CO., LTD., Tokyo 100-8321 (JP)
(72) Inventor: KAWASAKI, Hiroshi, Ichihara-shi, Chiba 2990107 (JP)
(74) Representative: Gille Hrabal
(86) International application number: PCT/JP2005/001216
(87) International publication number: WO 2005/073353

(56) References cited:
- EP-A1- 0 712 834
- JP-A- 8 259 980
- JP-A- 55 084 396
- JP-A- 2001 234 187
- JP-A- 2002 097 485
- JP-A- 2002 212 580
- JP-A- 2004 018 531
- US-A- 5 580 482
- US-A- 6 046 144

## Description

### TECHNICAL FIELD

The present invention relates to a biodegradable lubricating oil composition. More specifically, it relates to a synthetic ester-based biodegradable lubricating oil composition which has excellent biodegradability, a high viscosity index, a low pour point, a high flash point, being satisfactory with lubricity, oxidative stability, property of preventing the corrosion of iron and non-ferrous metals, and suitability for use with sealing materials.

### BACKGROUND ART

In recent years, considerable attention has been paid to a biodegradable lubricating oil in the field of lubricant application due to environmental pollution-control measures. Research and development was started and commercially available products were manufactured in this field from early 1990's in Japan. However, biodegradable lubricating oils have not widely been used in Japan because of their higher cost compared with conventional mineral oil-based lubricating oils, in spite of high attention. Japan is far behind European countries where use of a biodegradable lubricating oil is made compulsory by law.

Vegetable oils such as rapeseed oil, synthetic esters and polyalkyleneglycols have been used as a biodegradable base oil. However, vegetable oils have a problem of thermal or oxidative instability as well as unstable supply despite low cost, and polyalkyleneglycols have a problem of a poor suitability for use with sealing materials despite low cost and good thermal stability. Therefore, although synthetic esters are becoming more popular as biodegradable lubricating oils in Japan, they still have a substantial weakness against a mineral oil-based lubricating oil in terms of the cost and oxidative stability.

Japan Environment Association has authorization standard, named "ECOMARK", for biodegradable hydraulic fluids. The authorization standard was drastically revised in July, 1998 for further severe control. The major changes were as follows:
(1) The biodegradability standard was changed from the partial biodegradation test, "CEC Test Guideline" (reference degree of biodegradability: 67% or more) to the inherent biodegradation test, "OECD Test Guideline 301C method" (reference degree of biodegradability: 60% or more), and
(2) The acute toxicity test for Japanese medaka (Oryzias latipes), JIS K 0102 (reference: LC₅₀ ≥ 100 mg/L) was added.

The following examples of a biodegradable lubricating oil have been disclosed:
A lubricating oil composition comprising a polyol ester base oil composed of a carboxylic acid having 5 to 14 carbon atoms and a carboxylic acid having 15 to 38 carbon atoms in a weight ratio of 0.1:99.9 to 50:50, in which at least one of the compounds selected from the group consisting of a sulfonate, a condensate between an alkanolamine and a carboxylic acid having 5 to 14 carbon atoms and a polybutenyl succinimide is contained at 0.1 to 15 weight% (for example, Patent Document 1), a fire-resistant hydraulic fluid comprising a hydraulic base oil containing, as a main component, a polyol partial ester having a hydroxyl value of 35 mg KOH/g or more, a flash point of 290°C or more and a number-average molecular weight of 600 to 1500, wherein the ester is composed of a polyol having 3 to 12 carbon atoms and 3 to 6 total hydroxyl groups and a linear-chain monocarboxylic acid having 6 to 22 carbon atoms (for example, Patent Document 2), a lubricating oil comprising a synthetic ester having a kinematic viscosity of 20 to 40 mm²/s at 40°C, a viscosity index of 120 or more and a pour point of -30°C or less, wherein the ester is composed of a dimethylol alkane wherein the alkane has 5 to 7 carbon atoms and a linear-chain fatty acid having 10 to 20 carbon atoms (for example, Patent Document 3), a non-aqueous hydraulic fluid comprising a base oil composed of trimethylolpropane trioleate or neopentylglycol dioleate and a surfactant such as polyoxyethylene alkyl ether (for example, Patent Document 4) and the like.

Although the above-mentioned biodegradable lubricating oils are satisfactory with respect to lubricity and oxidative stability, they still have problems of a high pour point, substantial metal dissolution of non-ferrous metals used for materials for hydraulic machinery, Lubricant compositions which are stabilized against destruction through heat and oxygen are described in Patent Document 5. The document describes compositions made from a number of different components. A first component is a natural or synthetic oil component. One of the optional choices for such a natural or synthetic oil component is an ester compound containing methylol groups (column 8, lines 42 to 47). Furthermore, the composition contains additives, such as an antioxidant. Numerous phenolic antioxidants are mentioned, but other types of antioxidants are possible as well. Other additives are "other metal deactivators, other corrosion inhibitors, viscosity improvers, dispersants, detergents, extreme pressure and antiwear additives and pour-point depressants", see column 6, lines 9 to 12. In the group of the "dispersants/depressants" calcium sulfonates are mentioned (column 8, lines 64/65). The feature of the total base number is not mentioned. The examples are compositions containing a vegetable oil (canola oil or sunflower oil) and a phenolic antioxidant.
Lubricants containing polyol esters are described in Patent Document 6.
Antioxidant compositions which are useful for gear lubricating oils are described in Patent Document 7.

In the further Patent Documents 8 to 10 lubricating oil compositions are described

Patent Document 1: JP Kokai 1993-339591
Patent Document 2: JP Kokai 1994-228579
Patent Document 3: JP Kokai 1997-249889
Patent Document 4: JP kokai 1999-323373
Patent Document 5: US 5,580,482 A
Patent Document 6: EP 0 712 834 A1
Patent Document 7: US 6,046,144 A
Patent Document 8: JP 2002-097485 A
Patent Document 9: JP 08-259980 A
Patent Document 10: JP 2001-234187 A

### DISCLOSURE OF THE INVENTION

### PROBLEMS TO BE SOLVED BY THE INVENTION

The present invention was completed under these circumstances with an object to provide a biodegradable lubricating oil composition which has excellent biodegradability, a high viscosity index, a low pour point, a high flash point, being satisfactory with lubricity, oxidative stability, property of preventing the corrosion of iron and non-ferrous metals, and suitability for use with sealing materials.

### MEANS FOR SOLVING THE PROBLEMS

The present inventor studied intensively in order to develop a biodegradable lubricating oil composition which meets the aforementioned preferable properties, and found that a lubricating oil composition having a certain value or more of the biodegradability that is determined according to the OECD Test Guideline 301C method satisfies the purpose of the study, wherein the lubricating oil composition is composed of a synthetic ester base oil comprising mainly an ester composed of an aliphatic hindered polyol having a specific structure and an aliphatic monocarboxylic acid, to which a specific additive is admixed in a predetermined ratio. The present invention has been accomplished based on the aforementioned findings. That is, the present invention provides:
(1) A biodegradable lubricating oil composition comprising (A) a synthetic ester base oil comprising at least 50 mass% hindered ester of an aliphatic monocarboxylic acid with an aliphatic hindered polyol represented by the general formula (I): wherein R¹ and R² represent independently a hydrocarbon group having 1 to 6 carbon atoms or a methylol group, and n is an integer of 0 to 4; and (B) ingredients which are (a) 0.1 to 5.0 mass% phenolic antioxidant based on the total amount of the lubricating oil composition, (b) 0.01 to 2.0 mass% calcium sulfonate having a having a total base number in the range from 0 to 100 mg KOH/g based on the total amount of the lubricating oil composition, and (c) 0.01 to 1.0 mass% triazole compound based on the total amount of the lubricating oil composition, and having a degree of biodegradation of 70 % or higher when examined by the test for the degree of microbial degradation of chemical substances according to the OECD Test Guideline 301C method,
(2) The biodegradable lubricating oil composition according to the aforementioned (1), wherein the 96-h LC₅₀ value of the acute toxicity test for Japanese medaka (Oryzias latipes) according to the JIS K 0102 test method is 100 mg/L or more,
(3) The biodegradable lubricating oil composition according to the aforementioned (1) or (2), wherein the viscosity index determined according to the JIS K 2283 method is 130 or more, the pour point determined according to the JIS K 2269 method is -40°C or less, and the flash point determined by using the Cleveland Open Cup (COC) tester according to the JIS K 2265 method is 250°C or more,
(4) The biodegradable lubricating oil composition according to the aforementioned (1), wherein the aliphatic hindered polyol is at least one selected from neopentyl glycol; 2-ethyl-2-methyl-1-,3-propanediol; 2,2-diethyl-1,3-propanediol; trimethylolethane; trimethylolpropane; trimethylolbutane; trimethylolpentane; trimethylolhexane; trimethylolheptane; pentaerythritol; 2,2,6,6-tetramethyl-4-oxa-1,7-heptanediol; 2,2,6,6,10,10-hexamethyl-4, 8-dioxa-1,11-undecanediol; 2,2,6,6,10,10,14,14-octamethyl-4,8,12-trioxa-1,15-pentadecanediol; 2,6-dihydroxymethyl-2,6-dimethyl-4-oxa-1,7-heptanediol; 2,6,10-trihydroxymethyl-2,6,10-trimethyl-4,8-dioxa-1,11-undecanediol; 2,6,10,14-tetrahydroxymethyl-2,6,10,14-tetramethyl-4,8,12-trioxa-1,15-pentadecanedi ol; di(pentaerythritol); tri(pentaerythritol); tetra(pentaerythritol) and penta(pentaerythritol),
(5) The biodegradable lubricating oil composition according to any of the aforementioned (1) to m(4), wherein the aliphatic monocarboxylic acid is a saturated or unsaturated monocarboxylic acid having 6 to 22 carbon atoms,
(6) The biodegradable lubricating oil composition according to any of the aforementioned (1) to (3), wherein the hindered ester is at least one selected from an ester of a saturated or unsaturated monocarboxylic acid having 6 to 22 carbon atoms with pentaerythritol, and an ester of a saturated or unsaturated monocarboxylic acid having 6 to 22 carbon atoms with trimethylolpropane, and.
(7) The biodegradable lubricating oil composition according to any of the aforementioned (1) to (6), which contains 0.1 to 5.0 mass% of an extreme-pressure agent and/or an antiwear agent as a component (B) (d) based on the total amount of the lubricating oil composition.

### ADVANTAGES OF THE INVENTION

According to the present invention, there is provided a synthetic ester-based biodegradable lubricating oil composition which has excellent biodegradability, a high viscosity index, a low pour point, a high flash point, being satisfactory with lubricity, oxidative stability, property of preventing the corrosion of iron and non-ferrous metals, and suitability for use with sealing materials.

### BEST MODE FOR CARRYING OUT THE INVENTION

The biodegradable lubricating oil composition of the present invention comprises; (A) a synthetic ester base oil and (B) ingredients comprising a combination of (a) a phenolic antioxidant, (b) calcium sulfonate having a low base number and (c) a triazole compound.

The synthetic ester base oil used as component (A) of the present invention comprises at least 50 mass% hindered ester of an aliphatic monocarboxylic acid with an aliphatic hindered polyol which has one or more quaternary carbon atoms per molecule and in which at least one of the quaternary carbon atoms has one to four methylol groups bonded thereto.

The aliphatic hindered polyol which has one or more quaternary carbon atoms per molecule and in which at least one of the quaternary carbon atoms has one to four methylol groups bonded thereto of the present invention (which may be referred to simply as the hindered polyol hereinafter) is a compound represented by general formula (I):

(wherein R¹ and R² independently represent a hydrocarbon group having 1 to 6 carbon atoms or a methylol group, and n is an integer of 0 to 4.)

As the hydrocarbon group having 1 to 6 carbon atoms among R¹ and R² in general formula (I), a linear or branched alkyl or alkenyl group is preferable, and especially, an alkyl group is preferable.

The compound represented by general formula (I) (hindered polyols) refers to a hindered polyol such as neopentyl glycol, trimethylolalkane (the alkane has 2 to 7 carbon atoms) and pentaerythritol or a dehydrated condensate thereof. Specific examples include neopentyl glycol; 2-ethyl-2-methyl-1,3-propanediol; 2,2-diethyl-1,3-propanediol; trimethylolethane; trimethylolpropane; trimethylolbutane; trimethylolpentane; trimethylolhexane; trimethylolheptane; pentaerythritol; 2,2,6,6-tetramethyl-4-oxa-1,7-heptanediol; 2,2,6,6,10,10-hexamethyl-4,8-dioxa-1,11-undecanediol; 2,2,6,6,10,10,14,14-octamethyl-4,8,12-trioxa-1,15-pentadecanediol; 2,6-dihydroxymethyl-2,6-dimethyl-4-oxa-1,7-heptanediol; 2,6, 10-trihydroxymethyl-2,6, 10-trimethyl-4,8-dioxa-1,11-undecanediol; 2,6,10,14-tetrahydroxymethyl-2,6,10,14-tetramethyl-4,8,12-trioxa-1,15-pentadecanediol; di(pentaerythritol); tri(pentaerythritol); tetra(pentaerythritol); penta(pentaerythritol) and the like.

The hindered polyols may be used singly or as a mixture of 2 or more thereof in the esterification. In the above-described general formula (I), a preferable number of n is 0 to 2.

Preferred hindered polyols are trimethylolpropane, neopentyl glycol, pentaerythritol and dehydrated condensates thereof, wherein preferable dehydrated condensates are bimolecular or trimolecular condensates.

The above-described hindered polyols can be synthesized according to the conventional method. Also, the dehydrated condensates of the hindered polyols can be synthesized by dehydration condensation of the hindered polyols in the presence of a catalyst at about 180°C by heating the hindered polyols at a temperature above the melting point and dispersing them in a solvent.

On the other hand, as the aliphatic monocarboxylic acids used in the esterification of the aliphatic hindered polyols mentioned above, saturated or unsaturated monocarboxylic acids having 6 to 22 carbon atoms are used preferably. The acyl group of the monocarboxylic acids may be linear or branched. Examples of the aliphatic monocarboxylic acids include linear saturated monocarboxylic acids such as caproic acid, enanthic acid, caprylic acid, pelargonic acid, capric acid, undecanoic acid, lauric acid, tridecanoic acid, myristic acid, pentadecanoic acid, palmitic acid, heptadecanoic acid, stearic acid, nonadecanoic acid, arachic acid and behenic acid, linear unsaturated monocarboxylic acids such as undecenoic acid, oleic acid, elaidic acid, cetoleic acid, erucic acid, brassidic acid, linoleic acid and linolenic acid, branched saturated monocarboxylic acids such as isomyristic acid, isopalmitic acid, isostearic acid, 2,2-dimethylbutanoic acid, 2,2-dimethylpentanoic acid, 2,2-dimethyloctanoic acid, 2-ethyl-2,3,3-trimethylbutanoic acid, 2,2,3,4-tetramethylpentanoic acid, 2,5,5-trimethyl-2-t-butylhexanoic acid, 2,3,3-trimethyl-2-ethylbutanoic acid, 2,3-dimethyl-2-isopropylbutanoic acid, 2-ethylhexanoic acid and 3,5,5-trimethylhexanoic acid, and the like. The aliphatic monocarboxylic acids may be used singly or as a mixture of two or more kinds in the esterification.

The hindered ester synthesized by esterification reaction of the above-mentioned hindered polyol with the aliphatic monocarboxylic acid may be a fully-esterified or partially-esterified compound. A preferable hindered ester is the fully-esterified compound.

The hindered esters may be used singly or as a mixture of two or more thereof in the biodegradable lubricating oil composition of the present invention. Further, the amount of the hindered ester in the synthetic ester base oil is 50 mass% or more, preferably 70 mass% or more, and furthermore preferably 80 mass% or more in order to satisfy the predetermined properties of the biodegradable lubricating oil composition described below.

As a synthetic ester base oil which can be used together with the hindered ester, there may be cited an ester composed of an aliphatic polyol other than the hindered polyol mentioned above and the above-described monocarboxylic acid from the viewpoint of biodegradability, etc. of the lubricating oil composition.

Kinematic viscosity of the synthetic ester base oil used as the component (A) in the lubricating oil composition depends on the purpose of use of the lubricating oil composition, and is approximately in the range from 10 to 200 mm²/s at 40°C in general, preferably in the range from 10 to 100 mm²/s, and more preferably in the range from 15 to 80 mm²/s in the case of hydraulic fluid application.

An acid value of the synthetic ester base oil is preferably 3 mg KOH/g or less and particularly preferably 1 mg KOH/g or less in terms of prevention of corrosion of machinery. Further, there is no particular limitation for a hydroxyl value, but it is preferably 50 mg KOH/g or less and particularly preferably 20 mg KOH/g or less from a viewpoint of lubricity.

In the lubricating oil composition of the present invention, phenolic antioxidant as component (a) of the ingredient (B) is not particularly limited, and phenolic antioxidant known in the art can be used with suitable selection. Examples of the phenolic antioxidant include 4,4'-methylenebis(2,6-di-t-butylphenol); 4,4'-bis(2,6-di-t-butylphenol); 4,4'-bis(2-methyl-6-t-butylphenol); 2,2'-methylenebis(4-ethyl-6-t-butylphenol); 2,2'-methylenebis(4-methyl-6-t-butylphenol); 4,4'-butylidenebis(3-methyl-6-t-butylphenol); 4,4'-isopropylidenebis(2,6-di-t-butylphenol); 2,2'-methylenebis(4-methyl-6-t-nonylphenol); 2,2'-isobutylidenebis(4,6-dimethylpenol); 2,2'-methylenebis(4-methyl-6-cyclohexylphenol); 2,6-di-t-butyl-4-methylphenol; 2,6-di-t-butyl-ethylphenol; 2,4-dimethyl-6-t-butylphenol; 2,6-di-t-amyl-p-cresol; 2,6-di-t-butyl-4-(N,N'-dimethylaminomethylphenol), 4,4'-thiobis(2-methyl-6-t-butylphenol); 4,4'-thiobis(3-methyl-6-t-butylphenol); 2,2'-thiobis(4-methyl-6-t-butylphenol); bis(3-methyl-4-hydroxy-5-t-butylbenzyl)sulfide; bis(3,5-di-t-butyl-4-hydroxybenzyl)sulfide; n-octadecyl-3-(4-hydroxy-3,5-di-t-butylphenyl)propionate; 2,2'-thio[diethyl-bis-3-(3,5-di-t-butyl-4-hydroxyphenyl)propionate] and the like. Among them, those of bisphenol-based and ester-containing phenols are preferable.

In the present invention, these phenolic antioxidants may be used singly or in a combination of two or more thereof. The aforementioned hindered ester used for the synthetic ester base oil has satisfactory oxidative stability by itself, and the oxidative stability of the lubricating oil composition can further be improved by admixing such a phenolic antioxidant, which also results in the increase in thermal stability. The amount of the phenolic antioxidant added is in the range from 0.1 to 5.0 mass% based on the total amount of the present composition. When the amount of the phenolic antioxidant is in the range mentioned above, the effect of improvement in the oxidative stability is exhibited and the balance between cost and effectiveness becomes excellent. The preferable amount of the phenolic antioxidant admixed is in the range from 0.5 to 3.0 mass%. In addition, although the effect of improvement in the oxidative stability can be obtained by adding an amine-based antioxidant as well, the phenolic antioxidants are used in the present invention from a viewpoint of impact on ecosystems.

In the lubricating oil composition of the present invention, the low base number calcium sulfonate as the component (b) in the ingredient (B) is added to give anti-rust effect to the lubricating oil composition and has also detergency and dispersion function. The calcium sulfonate is a calcium salt of a sulfonated alkyl-substituted aromatic compound. When the base number of the calcium sulfonate is too large, its solubility in the synthetic ester base oil is not sufficient. Therefore, the calcium sulfonate having a low base number such that the total base number (TBN) is in the range from 0 to 100 mg KOH/g (preferably in the range from 0 to 50 mg KOH/g) is used in the present invention.

The low base number calcium sulfonates may be used singly or in a combination of two or more thereof. The amount of the calcium sulfonate added is in the range from 0.01 to 2.0 mass% based on the total amount of the composition. When the amount of the low base number calcium sulfonate is in the range described above, satisfactory rust-prevention effect can be exhibited and excellent balance between cost and effectiveness is obtained. The amount of the low base number calcium sulfonate is preferably in the range from 0.05 to 1.0 mass%.

In the lubricating oil composition of the present invention, the triazole compound as (c) component in the ingredient (B) is added as a metal deactivator and is used to give corrosion-prevention effect for non-ferrous metals to the lubricating oil composition. Examples of the triazole compounds are benzotriazole and its derivatives. The triazole compound may be used singly or in a combination of two or more kinds thereof. The amount of the triazole compound admixed is in the range from 0.01 to 1.0 mass% based on the total amount of the composition. When the amount of the triazole compound is in the aforementioned range, satisfactory corrosion-prevention effect can be exhibited and excellent balance between cost and effectiveness is obtained. The amount of the triazole compound admixed is preferably in the range from 0.05 to 0.5 mass%.

In the lubricating oil composition of the present invention, the base oil itself has a level of lubricity equivalent to that of a conventional mineral oil-based antiwear hydraulic fluid, and in order to further improve the lubricity, an extreme-pressure agent and/or an antiwear agent may be added.

As the extreme-pressure agent, sulfur-based or phosphorus-based extreme-pressure agents can be used. Examples of the sulfur-based extreme-pressure agent are sulfurized fats and oils, sulfurized fatty acids, sulfurized esters, polysulfides, sulfurized olefins, thiocarbamates, thioterpenes, dialkylthiodipropionates and the like. Among them, sulfurized fats and oils, polysulfides and sulfurized olefins are preferred.

Examples of the phosphorus-based extreme-pressure agent are phosphates, (mono-, di-, or tri-)thiophosphates, amine salts of acidic phosphates, amine salts of (mono-, or di-)thiophosphates, phosphites, (mono-, di-, or tri-)thiophosphites and the like.

On the other hand, examples of the antiwear agent are zinc dithiophosphate (ZnDTP), zinc dithiocarbamate (ZnDTC), sulfurized molybdenum dithiophosphate (MoDTP), sulfurized molybdenum dithiocarbamate (MoDTC), and the like.

The extreme-pressure agent or antiwear agent may be used singly or in a combination of two or more kinds thereof. Further, the total amount of these agents admixed is in the range from 0.1 to 5.0 mass% based on the total amount of the composition. When the amount of the extreme-pressure agent and/or antiwear agent is in the aforementioned range, improvement in the antiwear effect is exhibited and excellent balance between cost and effectiveness is obtained. The amount of the extreme-pressure agent and/or antiwear agent is preferably in the range from 0.5 to 3.0 mass%.

In addition to the above-described additives, other additives such as viscosity index improver, pour point depressant, ash-free dispersant, surfactant, anti-foaming agent, demulsifier and so on can be added in such a range of the amount that no drawback to the effect of the present invention is brought about.

The properties of the biodegradable lubricating oil composition of the present invention are explained below.

The degree of biodegradation of the lubricating oil composition as determined by the microbial degradation test of chemical substances according to the OECD Test Guideline 301C method is 70 % or more (the reference degree of biodegradability is 60 % or more), and has excellent biodegradability. Further, the 96-h LC₅₀ value of the acute toxicity test for Japanese medaka (Oryzias latipes) as determined according to the JIS K 0102 standard is usually 100 mg/L or more, and has low impact on living organisms. Therefore, it can be said that the lubricating oil composition is a very environmentally friendly lubricating oil.

Also, the viscosity index is usually 130 or more, preferably 140 or more, the pour point is -40°C or lower, preferably -45°C or lower, and the flash point is usually 250°C or higher, preferably 260°C or higher. The synthetic ester base oil of the aforementioned component (A) has a viscosity index of 130 or more by itself, so addition of a viscosity index improver to the present composition is usually not necessary.

The lubricating oil composition has such a low pour point as mentioned above so that machinery startability at lower temperatures is excellent with the present composition when it is used as a hydraulic fluid. Also, the present composition has such a high flash point as mentioned above so that it has high flame retardance and hence it belongs to the category of a safe combustible liquid having VG of 32 or more according to the Fire Service Law.

The biodegradable lubricating oil composition of the present invention has excellent biodegradability, low impact to ecosystems, a high viscosity index, a low pour point, a high flash point, being satisfactory with lubricity, oxidative stability, property of preventing the corrosion of non-ferrous metals, and suitability for use with sealing materials. It has thus an excellent balance of those different properties.

The lubricating oil composition is preferable, for example, as a hydraulic fluid that is a power transmission fluid used in power transmission, power control, shock absorption and the like in a hydraulic system such as hydraulic machinery or equipment, a lubricating oil for automobiles used in automatic transmission, buffer, driving machinery such as power steering, gears and the like, a metal-working oil for cutting, polishing or plasticizing, and the like.

### EXAMPLES

The present invention is further described by the following examples but not limited thereto.

In addition, properties of the lubricating oil composition in each example were determined by the following methods:
(1) General Properties:
   (a) Kinematic viscosity at 40°C: Determined according to JIS K 2283 test method.
   (b) Viscosity index: Determined according to JIS K 2283 test method.
   (c) Acid value: Determined according to JIS K 2501 test method.
   (d) Hydroxyl value: Determined by the pyridine-acetyl chloride method according to JIS K 0070 test method.
   (e) Flash point: Determined by using the Cleveland Open Cup (COC) tester according to JIS K 2265 test method.
   (f) Pour point: Determined according to JIS K 2269 test method.
   (g) Antirust performance: Determined according to JIS K 2510 test method, wherein the rust formation after 24 hours of the test initiation was inspected by visual observation using distilled water at 60°C.
(2) Biodegradability:
   The degree of biodegradation was determined according to the modified MTTI test method, OECD301C. According to the authorized standard of "ECOMARK" revised in July, 1998, the degree of biodegradation is required to be 60 % or more.
(3) Acute toxicity to fish:
   The half lethal concentration (LC₅₀) after 96 hours was determined according to JIS K 0102 test method using Japanese medaka (Oryzias latipes). According to the authorized standards of "ECOMARK" revised in July, 1988, the LC₅₀ value is required to be 100 mg/L or more.
(4) Lubricity:
   (a) Shell Four-ball EP test (ASTM D2783): The load wear index (LWI) was determined from the last non-seizure load (LNL) and weld load (WL) values under the conditions including 1800 rpm and room temperature. The higher the LWI value, the better the load resistance.
   (b) Shell Four-ball wear test (ASTM D2783): The wear spot size was determined under the conditions including 1200 rpm, load of 294 N, temperature of 50°C and 30 minute test duration.
   (c) FZG Scouring test: The load stage of scouring was determined according to ASTM D5182-91 test method under the conditions including 90°C, 1450 rpm, 15 minute test duration, using the A-type gear.
   (d) Vane pump test (according to ASTM D2882): The degree of wear of vane and cam ring was determined by using a vane-type pump (Vickers Inc., V-104C Pump) after 250 hour operation under the conditions including 65°C, 13.7 MPa, 1200 rpm, 60 L oil volume and a flow rate of about 25 L/min.
(5) Oxidative stability:
   (a) IOT:
      The relative kinematic viscosity at 40°C (kinematic viscosity after the test/kinematic viscosity before the test) was determined, wherein 300 mL of a sample oil filled in a cylinder (45 mm in diameter, 500 mm in length) was subjected to a test in the presence of copper and iron as a catalyst, under the conditions either at 130°C for 48 hours or at 150°C for 48 hours with air intake rate of 10 L/hour.
   (b) High pressure circulation test:
      The relative kinematic viscosity at 40°C (kinematic viscosity after the test/kinematic viscosity before the test) was determined after a test sample was subjected to a test under the following conditions:
         Pump type: (UCHIDA-REXROTH "A2FO-10/ 61R-PPB06"),
         Pump pressure: 35 MPa,
         Oil flow rate: 13.6 L/min,
         Oil temperature: 80°C,
         Air intake rate: 1 NL/h,
         Catalyst: Cu coil (1.6 mm in diameter, 60 m in length), and
         Test duration: 600 h.

      Further, in the test described above, durability test was performed without limiting the test duration to measure the time when either the relative kinematic viscosity reaches 1.1, or the acid value reaches 2.0 mg KOH/g, or the Millipore value reaches 10 mg/100 mL of the sample (wherein the Millipore value is defined as a weight of fine powdery residue obtained by filtering out the residue with 0.8 µm membrane filter by vacuum filtration, followed by washing with n-hexane and drying), from which the service life was determined.
(6) Corrosion prevention for non-ferrous metals:
   After conducting a high-pressure circulation test for 600 hours in the manner similar to the aforementioned test (5), amounts of copper (dissolved from the catalyst) and zinc (dissolved from the piping material) in the sample oil were measured. In parallel to this method, a metal immersion test was also carried out according to the following procedure:
      (a) Put 100 g of a sample oil in a 200 mL mayonnaise bottle,
      (b) Weigh the test piece after polishing with sandpaper #240, washing with gasoline and drying,
      (c) Put one test piece into one sample bottle and heat at 100°C for 168 hours in a temperature-controlled bath,
      (d) Take out the test piece, wipe off the sample oil on the test piece using waste cloth, wash with gasoline, dry and weigh.

      At this time, a metal immersion test as described above was carried out on a zinc test piece (1.0 mm × 26 mm × 60 mm) for the oil sample used in Comparative example 6, a weight loss of 0.47 % was observed.
   (7) Suitability for use with sealing material:
      An immersion test was performed according to the JIS K 6258 method for nitrile-butadiene rubber (NBR) and polyurethane at 100°C for 240 hours and at 120°C for 240 hours, respectively, and the rate of change after the test with respect to values before the test was determined for each property: [mass change rate (%),
      volume change rate (%), hardness change (no units), change rate of tensile strength (%), and change rate of elongation at break (%)].
      Here, judgment criteria for evaluation of each of the aforementioned properties are as follows:
         ⊚ (excellent), ○(good), Δ (normal), and × (poor).

Examples 1 to 3 and Comparative examples 1 to 8
(1) Lubricating oil compositions with compositions shown in Tables 1-1 and 1-2 were prepared along with commercially-available products. General properties and biodegradability of these lubricating oil compositions are listed in Tables 2-1 and 2-2.
Table 1

**Table 1-1**

| | | Examples | | | Comparative examples | | |
|---|---|---|---|---|---|---|---|
| | | 1 | 2 | 3 | 1 | 2 | 3 |
| Prepared product or commercial product | | Prepared oil | Prepared oil | Prepared oil | Commercial oil A | Commercial oil B | Commercial oil C |
| Type of base oil | | Ester | Ester | Ester | Ester | Ester | Ester |
| Base oil (mass%) | Hindered ester | PET Ester 31.6 | TMP Ester 50.1 | TMP Ester 90.8 | NPG dioleate 2.0 parts | NPG dioleate 3.0 parts | - |
| | | TMP trioleate 66.2 | TMP trioleate 47.2 | TMP trioleate 6.5 | TMP trioleate 8.0 parts | TMP trioleate 8.0 parts | - |
| | | - | - | - | - | PET tetraoleate 1.0 part | - |
| | Non-hindered ester | - | - | | Aliphatic ester | Aliphatic ester | Rapeseed oil |
| | Total | 97.8 | 97.3 | 97.3 | | | |
| Antioxidant (mass%) | | Phenolic 1.4 | Phenolic 1.4 | Phenolic 1.4 | Phenolic | Amine-based | Phenolic |
| Antirust agent (mass%) | | Low base number Ca sulfonate 0.1 | Low base number Ca sulfonate 0.1 | Low base number Ca sulfonate 0.1 | - | - | - |
| Metal deactivator (mass%) | | Benzotriazole-based 0.1 | Benzotriazole-based 0.1 | Benzotriazole-based 0.1 | - | - | - |
| Extreme-pressure agent or antiwear agent (mass%) | | - | S, P type 10 | S, P type 1.0 | ZnDTP | Oleic acid, P type | Oleic acid, P type |
| Other additives (mass%) | | Methacrylate anti-foaming agent 0.6 | Anti-foaming agent 0.1 | Anti-foaming agent 0.1 | Large base-number Ca sulfonate, imide-based friction modifier | POE alkylether | - |

Table 2

**Table 1-2**

| | | Comparative examples | | | | |
|---|---|---|---|---|---|---|
| | | 4 | 5 | 6 | 7 | 8 |
| Prepared product or commercial product | | Commercial oil D | Commercial oil E | Commercial oil F | Prepared oil | Commercial oil G |
| Type of base oil | | Ester | Ester | Ester | Ester | Mineral oil-based |
| Base oil (mass%) | Hindered ester | - | TMP isostearate, oleate (partially-esterified) | 2-butyl-2-ethyl-1,3-prop ane diol laurate and oleate mixture | TMP trioleate 98.85 | - |
| | | - | | | - | - |
| | | - | | | - | - |
| | Non-hindered ester | Diisotridecyladipate | - | - | - | - |
| | Total | | | | 98.85 | |
| Antioxidant (mass%) | | Amine-based | Amine-based 1.0 | Phenolic | Amine-based 1.0 | Phenolic, amine-based |
| Antirust agent (mass%) | | - | Low base number Ca sulfonate 0.1 | - | Low base number Ca sulfonate 0.1 | Polyol alkenyl succinate |
| Metal deactivator (mass%) | | - | Benzotriazole-based 0.05 | - | Benzotriazole-based 0.05 | Triazole-based |
| Extreme-pressure agent or antiwear agent (mass%) | | S, P type | - | Oleic acid | - | Tricresyl phosphate |
| Other additives (mass%) | | Polybutene polymer | Polymethacrylate | - | - | Various additives*1 1 |

| | | | | | | |
|---|---|---|---|---|---|---|
| *1 Various additives: a pour point depressant, detergent dispersant, anti-foaming agent, demulsifier, etc. | | | | | | |

Note:
In Tables 1-1 and 1-2, PET denotes pentaerythritol, TMP denotes trimethylolpropane, NPG denotes neopentyl glycol, ZnDTP denotes zinc dithiophosphate, and POE denotes polyoxyethylene.
Table 3 Table 4
(2) Tables 3-1 and 3-2 indicate the test results of lubricity, oxidative stability and corrosion prevention of non-ferrous metals for each lubricating oil composition. Table 5 Table 6
(3) Table 4 indicates the test results of suitability for use with sealing materials of the lubricating oil composition of Example 1 and the lubricating oil compositions of Comparative examples I to 4.
Table 7

As is evident from the results of Tables 1 to 4, the lubricating oil compositions of the present invention (Examples 1 to 3) have a well-balanced properties such as excellent biodegradability, a high viscosity index, a low pour point, a high flash point, being satisfactory with lubricity, oxidative stability, property of preventing the corrosion of iron and non-ferrous metals, and suitability for use with sealing materials.

### INDUSTRIAL APPLICABILITY

The biodegradable lubricating oil composition of the present invention comprises a synthetic ester base oil having excellent biodegradability, has well-balanced properties including lubricating performance, and is preferably used, for example, as a hydraulic fluid, automotive lubricating oil, metal-working oil, and so on.

## Claims

1. A biodegradable lubricating oil composition comprising
(A) a synthetic ester base oil comprising at least 50 mass% hindered ester of an aliphatic monocarboxylic acid with an aliphatic hindered polyol represented by the general formula (I): wherein R¹ and R² represent independently a hydrocarbon group having 1 to 6 carbon atoms or a methylol group, and n is an integer of 0 to 4; and
(B) ingredients which are
(a) 0.1 to 5.0 mass% phenolic antioxidant based on the total amount of the lubricating oil composition,
(b) 0.01 to 2.0 mass% calcium sulfonate having a total base number in the range from 0 to 100 mg KOH/g based on the total amount of the lubricating oil composition, and
(c) 0.01 to 1.0 mass% triazole compound based on the total amount of the lubricating oil composition, and
having a degree of biodegradation of 70 % or higher when examined by the test for the degree of microbial degradation of chemical substances according to the OECD Test Guideline 301C method.

2. The biodegradable lubricating oil composition according to claim 1, wherein the 96-h LC₅₀ value of the acute toxicity test for Japanese medaka (Oryzias latipes) according to the JIS K 0102 test method is 100 mg/L or more.

3. The biodegradable lubricating oil composition according to claim 1 or 2, wherein the viscosity index determined according to the JIS K 2283 method is 130 or more, the pour point determined according to the JIS K 2269 method is -40°C or less, and the flash point determined by using the Cleveland Open Cup (COC) tester according to the JIS K 2265 method is 250°C or more.

4. The biodegradable lubricating oil composition according to Claim 1, wherein the aliphatic hindered polyol is at least one selected from neopentyl glycol; 2-ethyl-2-methyl-1,3-propanediol; 2,2-diethyl-1,3-propanediol; trimethylolethane; trimethylolpropane; trimethylolbutane; trimethylolpentane; trimethylolhexane; trimethylolheptane; pentaerythritol; 2,2,6,6-tetramethyl-4-oxa-1,7-heptanediol; 2,2,6,6,10,10-hexamethyl-4,8-dioxa-1,11-undecanediol; 2,2,6,6,10,10,14,14-octamethyl-4,8,12-trioxa-1,15-pentadecanediol; 2,6-dihydroxymethyl-2,6-dimethyl-4-oxa-1,7-heptanediol; 2,6,10-trihydroxymethyl-2,6,10-trimethyl-4,8-dioxa-1,11-undecanediol; 2,6,10,14-tetrahydroxymethyl-2,6,10,14-tetramethyl-4,8,12-trioxa-1,15-pentadecanediol; di(pentaerythritol); tri(pentaerythritol); tetra(pentaerythritol) and penta(pentaerythritol).

5. The biodegradable lubricating oil composition according to any of claims 1 to 4, wherein the aliphatic monocarboxylic acid is a saturated or unsaturated monocarboxylic acid having 6 to 22 carbon atoms.

6. The biodegradable lubricating oil composition according to any of claims 1 to 3, wherein the hindered ester is at least one selected from an ester of a saturated or unsaturated monocarboxylic acid having 6 to 22 carbon atoms with pentaerythritol, and an ester of a saturated or unsaturated monocarboxylic acid having 6 to 22 carbon atoms with trimethylolpropane.

7. The biodegradable lubricating oil composition according to any of claims 1 to 6, which contains 0.1 to 5.0 mass% of an extreme-pressure agent and/or an antiwear agent as a component (B) (d) based on the total amount of the lubricating oil composition.

## Patentansprüche

1. Biologisch abbaubare Schmierölzusammensetzung, umfassend:
(A) ein synthetisches Öl auf Esterbasis, welches mindestens 50 Massen-% eines gehinderten Esters einer aliphatischen Monocarbonsäure mit einem aliphatischen gehinderten Polyol nach der allgemeinen Formel (I): worin R¹ und R² jeweils unabhängig eine Kohlenwasserstoffgruppe mit 1 bis 6 Kohlenstoffatomen oder eine Methylolgruppe sind, und n eine ganze Zahl von 0 bis 4 ist; und
(B) Inhaltsstoffe, bei denen es sich um
(a) 0,1 bis 5,0 Massen-% phenolisches Antioxidationsmittel, bezogen auf die Gesamtmenge der Schmierölzusammensetzung,
(b) 0,01 bis 2,0 Massen-% Calciumsulfonat mit einer Gesamtbasenzahl im Bereich von 0 bis 100 mg KOH/g, bezogen auf die Gesamtmenge der Schmierölzusammensetzung, und
(c) 0,01 bis 1,0 Massen-% einer Triazol-Verbindung, bezogen auf die Gesamtmenge der Schmierölzusammensetzung, handelt, und
wobei die Schmierölzusammensetzung einen Bio-Abbaubarkeitsgrad von 70 % oder mehr aufweist, wenn dieser anhand der Prüfung des mikrobiologischen Abbaubarkeitsgrads chemischer Substanzen nach dem Verfahren in den OECD Prüfrichtlinien 301C ermittelt wird.

2. Die biologisch abbaubare Schmierölzusammensetzung nach Anspruch 1, wobei der 96h-LC₅₀-Wert bei Prüfung der akuten Toxizität für den japanischen Medaka (Oryzias latipes) nach dem JIS K 0102 Prüfverfahren 100 mg/L oder mehr beträgt.

3. Die biologisch abbaubare Schmierölzusammensetzung nach Anspruch 1 oder 2, wobei der Viskositätsindex, der nach dem JIS K 2283 Verfahren bestimmt wird, 130 oder mehr ist, der Fließpunkt, der nach dem JIS K 2269 Verfahren bestimmt wird, -40°C oder weniger ist und der Flammpunkt, der mittels eines Prüfgeräts für das Cleveland-Verfahren im offenen Tiegel nach dem JIS K 2265 Verfahren bestimmt wird, 250 °C oder mehr ist.

4. Die biologisch abbaubare Schmierölzusammensetzung nach Anspruch 1, wobei das aliphatische gehinderte Polyol mindestens ein Polyol ist, das aus Neopentylglykol; 2-Ethyl-2-methyl-1,3-propandiol; 2,2-Diethyl-1,3-propandiol; Trimethylolethan; Trimethylolpropan; Trimethylolbutan; Trimethylolpentan; Trimethylolhexan; Trimethylolheptan; Pentaerythritol; 2,2,6,6-Tetramethyl-4-oxa-1,7-heptandiol; 2,2,6,6,10,10-Hexamethyl-4,8-dioxa-1,11-undecandiol; 2,2,6,6,10,10,14,14-Octamethyl-4,8,12-trioxa-1,15-pentadecandiol; 2,6-Dihydroxymethyl-2,6-dimethyl-4-oxa-1,7-heptandiol; 2,6,10-Trihydroxymethyl-2,6,10-trimethyl-4,8-dioxa-1,11-undecandiol; 2,6,10,14-Tetrahydroxymethyl-2,6,10,14-tetramethyl-4,8,12-trioxa-1,15-pentadecandiol; Di(pentaerythritol); Tri(pentaerythritol); Tetra(pentaerythritol); Penta(pentaerythritol) ausgewählt wird.

5. Die biologisch abbaubare Schmierölzusammensetzung nach einem der Ansprüche 1 bis 4, wobei die aliphatische Monocarbonsäure eine gesättigte oder ungesättigte Monocarbonsäure mit 6 bis 22 Kohlenstoffatomen ist.

6. Die biologisch abbaubare Schmierölzusammensetzung nach einem der Ansprüche 1 bis 3, wobei der gehinderte Ester mindestens ein Ester ist, der aus einem Ester einer gesättigten oder ungesättigten Monocarbonsäure mit 6 bis 22 Kohlenstoffatomen mit Pentaerythritol und einem Ester einer gesättigten oder ungesättigten Monocarbonsäure mit 6 bis 22 Kohlenstoffatomen mit Trimethylolpropan ausgewählt wird.

7. Die biologisch abbaubare Schmierölzusammensetzung nach einem der Ansprüche 1 bis 6, welche 0,1 bis 5,0 Massen-% eines Extremdruckmittels und/oder eines Antiverschleißmittels als Komponente (B) (d), bezogen auf die Gesamtmenge der Schmierölzusammensetzung, enthält.

## Revendications

1. Composition d'huile de lubrification biodégradable comprenant
(A) une huile à base d'ester synthétique comprenant au moins 50% en masse d'ester encombré d'un acide monocarboxylique aliphatique avec un polyol aliphatique encombré représenté par la formule générale (I) : dans laquelle R¹ et R² représentent indépendamment un groupe hydrocarboné ayant 1 à 6 atome(s) de carbone ou un groupe méthylol, et n est un nombre entier allant de 0 à 4 ; et
(B) des ingrédients qui sont
(a) 0,1 à 5,0% en masse d'antioxydant phénolique par rapport à la quantité totale de la composition d'huile de lubrification,
(b) 0,01 à 2,0% en masse de sulfonate de calcium ayant un indice de basicité totale dans la plage allant de 0 à 100 mg KOH/g par rapport à la quantité totale de la composition d'huile de lubrification, et
(c) 0,01 à 1,0% en masse de composé triazole par rapport à la quantité totale de la composition d'huile de lubrification, et
ayant un degré de biodégradation supérieur ou égal à 70% lorsqu'elle est soumise au test du degré de dégradation microbienne des substances chimiques selon le procédé de la ligne directrice d'essais 301C de l'OCDE.

2. Composition d'huile de lubrification biodégradable selon la revendication 1, dans laquelle la valeur LC₅₀ à 96-h du test de toxicité aiguë pour le medaka Japonais (Oryzias latipes) selon le procédé d'essai JIS K0102 est supérieure ou égale à 100 mg/L.

3. Composition d'huile de lubrification biodégradable selon la revendication 1 ou 2, dans laquelle l'indice de viscosité déterminé selon le procédé JIS K2283 est supérieur ou égal à 130, le point d'écoulement déterminé selon le procédé JIS K2269 est inférieur ou égal à -40°C, et le point d'éclair déterminé en utilisant l'appareil Cleveland à vase ouvert (COC) selon le procédé JIS K2265 est supérieur ou égal à 250°C.

4. Composition d'huile de lubrification biodégradable selon la revendication 1, dans laquelle le polyol aliphatique encombré est au moins un élément choisi parmi le néopentylglycol ; le 2-éthyl-2-méthyl-1,3-propanediol ; le 2,2-diéthyl-1,3-propanediol ; le triméthyloléthane ; le triméthylolpropane ; le triméthylolbutane ; le triméthylolpentane ; le triméthylolhexane ; le triméthylolheptane ; le pentaérythritol ; le 2,2,6,6-tétraméthyl-4-oxa-1,7-heptanediol ; le 2,2,6,6,10,10-hexaméthyl-4,8-dioxa-1,11-undécanediol ; le 2,2,6,6,10,10,14,14-octaméthyl-4,8,12-trioxa-1,15-pentadécanediol ; le 2,6-dihydroxyméthyl-2,6-diméthyl-4-oxa-1,7-heptanediol ; le 2,6,10-trihydroxyméthyl-2,6,10-triméthyl-4,8-dioxa-1,11-undécanediol ; le 2,6,10,14-tétrahydroxyméthyl-2,6,10,14-tétraméthyl-4,8,12-trioxa-1,15-pentadécanediol ; le di(pentaérythritol) ; le tri(pentaérythritol) ; le tétra(pentaérythritol) et le penta(pentaérythritol).

5. Composition d'huile de lubrification biodégradable selon l'une des revendications 1 à 4, dans laquelle l'acide monocarboxylique aliphatique est un acide monocarboxylique saturé ou insaturé ayant 6 à 22 atomes de carbone.

6. Composition d'huile de lubrification biodégradable selon l'une des revendications 1 à 3, dans laquelle l'ester encombré est au moins un ester choisi parmi un ester d'un acide monocarboxylique saturé ou insaturé ayant 6 à 22 atomes de carbone avec du pentaérythritol et un ester d'un acide monocarboxylique saturé ou insaturé ayant 6 à 22 atomes de carbone avec du triméthylolpropane.

7. Composition d'huile de lubrification biodégradable selon l'une des revendications 1 à 6, qui contient 0,1 à 5,0% en masse d'un agent extrême pression et/ou d'un agent anti-usure en tant que composant (B)(d) par rapport à la quantité totale de la composition d'huile de lubrification.
